

No. 821,189.

PATENTED MAY 22, 1906.

J. A. POTTER.  
PROCESS OF SMELTING ORES.  
APPLICATION FILED JUNE 27, 1905.

2 SHEETS—SHEET 1.

FIG. 1



**WITNESSES:**

Paul Hoffman  
Leon Barlow

INVENTOR:

John A. Potter  
By Fred Wright  
Attorney.

No. 821,189.

PATENTED MAY 22, 1906.

J. A. POTTER.

## PROCESS OF SMELTING ORES.

APPLICATION FILED JUNE 27, 1905.

2 SHEETS--SHEET 2.

FIG. 3



FIG. 4



FIG. 2



**WITNESSES:**

Julie Grjebin  
Leon Boillot

*INVENTOR:*

John S. Potter  
By F. W. Wright,  
Attorney.

# UNITED STATES PATENT OFFICE.

JOHN A. POTTER, OF SAN FRANCISCO, CALIFORNIA.

## PROCESS OF SMELTING ORES.

No. 821,189.

Specification of Letters Patent.

Patented May 22, 1906.

Application filed June 27, 1905. Serial No. 267,302.

*To all whom it may concern:*

Be it known that I, JOHN A. POTTER, a citizen of the United States, residing at San Francisco, in the county of San Francisco and State of California, have invented certain new and useful Improvements in Processes of Smelting Ores, of which the following is a specification.

This invention relates to an improved process of smelting ores, particularly ferriferous ores, the object being to provide a process by which, first, the smelting may be conveniently accomplished on a large scale with the use of fluid fuels, such as petroleum-oils or fuel-gas; secondly, with which a compact and economical apparatus may be used; thirdly, in which the operation may be substantially continuous, and, fourthly, in which the cost of smelting shall be reduced to a minimum, principally from the economical proportioning and application of the amounts of fuel used, respectively, for reducing the oxids and for the application of the heat of fusion.

25 In the accompanying drawings, Figure 1 is a vertical section of the apparatus. Fig. 2 is a similar view at right angles to Fig. 1. Fig. 3 is a horizontal section on the line 3 3 of Fig. 1. Fig. 4 is a horizontal section on 30 the line 4 4 of Fig. 1.

Referring to the drawings, 1 represents a rectangular iron casing inclosing two regenerative chambers 2, provided with shelves 3 of fire-brick. Said chambers communicate 35 at the bottom with flues 4, leading to a stack 5, suitable reversing-dampers and air-inlet valves 6, such as is common in the art, being provided for changing the direction of the ingoing air and outflowing gases. Between 40 said regenerative chambers 2 is located a circular smelting-chamber 7 of fire-brick, the bottom of which is preferably formed of magnesite, over which pass the products of combustion. For said combustion fluid fuel, 45 such as petroleum-oil or fuel-gas, is admitted through pipes 8, discharging into the air or gas conduits 9, leading from the tops of said regenerative chambers 2 to said open-hearth combustion or smelting-chamber 7. At the 50 sides of said casing 1 are secured channel-posts 10, which are connected by channel-beams 11, across the mediate portions of which are secured transverse channel-beams 12, to which are secured angle-iron brackets 55 14, which in turn are secured to the metallic

casing 15 of a retort. To the lower end of said retort-casing 15 is secured a metal ring 16, which serves the purpose of supporting the brickwork 17 of said retort, said brick-work consisting of an inner cylindrical wall 60 18, an outer cylindrical wall 19, and ribs 20 connecting said walls for strengthening purposes and extending to a point near the top of the retort. The spaces 21 between these walls 18 19 and the ribs 20 serve as flues 65 through which the necessary hot gases from the combustion-chamber 7 pass, thereby highly heating said retort. Between the circular top 22 of the open hearth or smelting-chamber 7 and the ring-casting 16 is built a 70 roof or dome 23 of refractory material, as fire-brick, the top of said dome being separated from said ring-casting only by means of a water-cooled metallic top made in sections, as boxes 24, which can be separately 75 withdrawn when necessary for the purpose of inspection or repairs. This withdrawal is permissible by the fact that the retort does not rest upon said boxes 24, but is supported by the ring-casting 16 and the metal casing 80 15, which is in turn supported upon the channel-beams 13. Thus the necessary portion of the hot gases proceeding from the combustion-chamber 7, especially those from the extreme top thereof, are allowed to escape 85 through holes 25 through said water-cooled boxes and ring-casting, and thence to pass into the flues 21 of the retort to the top thereof, from any portion of which they can pass by the flue 26 to the main stack, the damper 90 27 being used to regulate the desired amount of gases to pass through the retort-flues 21.

Upon the top of the retort is supported a hopper and dependent ring 28, into which the material can be discharged by any suitable 95 means, as by cars moving upon rails 29, suitably supported upon a frame 30. In the middle of this frame is also mounted immediately over the hopper a vertical hydraulic cylinder 31, the piston 32 of which is connected with a plunger 33, which can pass through the mouth of the hopper and fit with sufficient closeness therein to substantially prevent gases escaping from the retort-chamber. When it is desired to charge the retort, 100 the plunger 33 is raised and the material which has been fed into the hopper falls into the dependent ring in the retort-chamber on the top of the previous charge. From the top of the retort-chamber pipes 34 convey 105 110

the gases distilled therefrom to the conduits 8, where they are burned with the fuel supplied through the pipes 8.

35 is a tap-hole for drawing off the molten metal and slag at suitable intervals, discharging the same into a separator 36, from which the slag and metal are withdrawn at different levels and disposed of.

When manufacturing cast-iron, as pig-iron, the process is as follows: The ores to be reduced, also suitable quantities of limestone and tarry carbonaceous material, are all brought to a pulverulent or granular condition and are thoroughly commingled. On first commencing the process, which when once started can be continued indefinitely, a shell, preferably of sheet metal of the same outside diameter as the interior of the retort, is inserted in the lower end of said retort, from which it extends to the bottom of the furnace-hearth, thus connecting the lower end of the retort and furnace-bottom. The above mixture is discharged into the retort to fill said shell, and then heat is applied to the outside of said shell by the combustion of liquid fuel admitted through the pipes 8, said shell being slowly subjected to the increasing heat of the liquid fuel, causing its contained mixture to become bound together and hardened by the oozing and charring of the tar and the coking of the combined carbon, after which it is melted at its lower end, at which time the heat in the furnace has been raised to such a degree that the continuous smelting process has commenced independent of any such extraneous means as that of the shell. The heat to which the mixture discharged into the retort is subjected increases gradually as the material descends, and the effect of this heat applied on the outside of the column of the mixture is to first char the tar and coke the combined carbon which forms a constituent of the outer layer or surface of the column, thus forming a hard binding crust or shell of carbon, lime, and ores bound together, which crust or shell gradually increases in thickness as the material descends into the lower and hotter zones of the retort, where the charring and coking operation extends into the interior of the column. The effect of this earlier charring process is to drive off the light hydrocarbon gases from the column of commingled pulverized ores, limestone, and carbonaceous material, said gases passing to the top of the retort, whence they are conveyed through the pipes 34 to the conduits 9 and are added to the fluid fuel used for smelting and heating purposes. During the intermediate and later process of charring, binding, and coking the hydrocarbon gases distilled from the carbonaceous material act as reducing agents on the ores commingled with said material, this reduction increasing as the heat becomes greater, since hotter

gases are distilled from the charred tar and combined carbon-coke of the column. Said gases oozing from the interior pass through the porous, hard, and charred column and escape to the top of the retort; but as the material in its descent approaches the bottom portion of the retort the gases so distilled, following the path of least resistance, tend to escape downward into the furnace and combustion-chamber proper and are there burned, the products of combustion passing up through the flues of the retort, highly heating the same, and finally out to the stack. Such hot reducing-gases constantly passing from the interior to the exterior of the column maintain a protection of the semimetallic particles that have formed on the exterior of the column from oxygen and oxidation during their exposure while traveling from the bottom of the retort through the furnace-chamber to the hottest part of the furnace, which is greatest just above the surface of the bath, at which point the heat completes the reduction of the ores, compelling the remaining oxygen thereof to unite with the solid carbon contained in the column, while at the same time the lime has combined with the silicious and other earths of the column, forming a slag which gathers and floats on the top of the metallic bath contained in the furnace-hearth. While this action is going on continuously, the metallic particles formed in the earlier stages of the process are constantly being attracted and fused together and formed into a contracted fibrous metallic column intermingled with entrapped combined carbon, as coke, from the carbonaceous material which gradually descends with the metallic column into and under the liquid bath of dissolving carbonaceous molten iron that is always maintained in the furnace-hearth, where they are constantly being dissolved and amalgamated in said bath. The accumulating molten iron and slag are tapped off at suitable intervals into a metal and slag separator located on the outside of the furnace-hearth, from where the metals and slags are drawn from different levels for final distribution. If the column should not gradually descend in the retort by its own gravity, it may be assisted from time to time by means of the plunger 33.

The carbonaceous material to be used as a binding, reducing, and recarbonizing agent to be mixed with the ores and lime includes various materials—such as residuum, asphaltum, coke, coal, charcoal, graphite, &c.—or it may be advantageous to mix any of the dry carbons with residuum, asphaltum, or oils, or the like. The object of using a tarry carbonaceous material is for two purposes, first, the contained tarry substances, which expand and ooze throughout the column of materials and as it is heated become charred, and thus, together with the coke re-

sulting from the coking of the fixed carbon, form a strong carbonaceous binder that binds the mass together, thus forming a column strong enough to withstand the downward and outward pressure of the superimpending portion thereof during the smelting process; secondly, the hot reducing carbonaceous gases generated from the charring and coking carbonaceous material at the different temperatures always act as an oxygen-consumer, ore-reducer, metallic protector, and metal-recarbonizer throughout the whole process of heating, binding, charring, smelting, and dissolving.

The result of the commingling of the combined carbon entrapped in the iron column as it is descending and being immersed in the liquid bath is that a continual replenishment takes place of carbon in the liquid bath, this being necessary to keep the liquid bath of the same constituency the same as that of pig-iron—that is, a carbonaceous iron containing sufficient carbon to furnish a solvent for the iron continually added thereto, increasing the fluidity of the iron, and maintaining its solvent effect. No mention has heretofore been made of any ferriferous ore except the ordinary iron ore; but the same process is applicable to a mixture of ores necessary to produce any grade of metal desired. Thus any kind of ferreous combination can be made by this process by adding the necessary ingredients, as ores, metals, or metaloids—for instance, a ferric manganese or spiegeleisen or chromic metals, &c.

The constant generation of the reducing carbon gases forms a very important part of the process, and a tarry carbonaceous material furnishes these gases at all temperatures of the process, as well as furnishes a strong binding material and solid carbon for final reduction and the recarbonizing of the liquid bath. Carbon gases do most of the oxygen-consuming in the early and intermediate stages of the process.

It is to be understood that my invention includes the application of this process as applied to other metals than iron so far as it may be found applicable thereto.

I claim—

1. The process of smelting ores which consists in mixing the ore with a material which when heated forms with said ore a binder, passing the mixture downward through an open-bottomed retort, subjecting the mixture to a gradually-increasing heat as it passes through the retort, whereby the body of material so subjected is hardened to prevent collapse, and applying a melting heat to

the material emerging from said retort, substantially as described.

2. The process of smelting iron ore, which consists in mixing the ore with suitable quantities of limestone and hydrocarbonaceous material, passing the mixture so formed through a retort, gradually increasing the heat applied to said material as it passes through the retort, thereby charring, coking and hardening the body of material, and applying a melting heat to the material emerging from the retort, substantially as described.

3. The process of smelting iron ore, which consists in reducing the ore, together with suitable quantities of limestone and hydrocarbonaceous material, to a finely-divided condition and commingling the same, passing the mixture so formed into and through a retort, applying heat to the mixture increasing gradually as it passes through the retort to 80 gasify, char and coke the hydrocarbonaceous material therein, applying products of combustion of fluid fuel to the exterior of the mixture to smelt the ore, drawing off the molten iron and slag at suitable intervals at 85 one end of the apparatus and adding fresh material at suitable intervals at the other end of the apparatus, in a continuous process, substantially as described.

4. The process of smelting iron ore, which 90 consists in finely dividing the ore and suitable quantities of limestone and hydrocarbonaceous material and commingling the same, applying heat to the mixture to distil hydrocarbon gases therefrom and form a hard 95 self-supporting column, and projecting such hard column into the path of products of combustion to reduce and melt the metallic substances therein, substantially as described.

5. The process of smelting iron ore, which 100 consists in reducing said ore, together with suitable quantities of limestone and tarry carbonaceous material, to a finely-divided condition and then commingling the same, continually feeding the mixture in proximity to 105 increasing heats to form a hard column continually projecting said column into the path of products of combustion to reduce and melt the ore and metallic substances therein, and drawing off at suitable intervals the molten 110 iron and slag, substantially as described.

In witness whereof I have hereunto set my hand in the presence of two subscribing witnesses.

JOHN A. POTTER.

Witnesses:

FRANCIS M. WRIGHT,  
BESSIE GORFINKEL.